# EUROPEAN PATENT SPECIFICATION

(11) **EP 3 109 300 B1**
(45) Date of publication and mention of the grant of the patent: **08.01.2020**
(21) Application number: 15751845.7
(22) Date of filing: 18.02.2015
(51) Int. Cl.: C10M 169/04, C10M 107/50, C10M 125/10, C10N 10/04, C10N 10/12, C10N 20/00, C10N 30/06, C10N 40/04, C10N 50/10

(54) **SILICONE GREASE COMPOSITION**
SILIKONFETTZUSAMMENSETZUNG
COMPOSITION DE GRAISSE DE SILICONE

(30) Priority: 18.02.2014 JP 2014028681
(43) Date of publication of application: 28.12.2016
(73) Proprietor: Kyodo Yushi Co., Ltd., Kanagawa 251-8588 (JP)
(72) Inventor: HIROOKA, Iwaki, Fujisawa-shi, Kanagawa 251-8588 (JP); YOSHINARI, Terasu, Fujisawa-shi, Kanagawa 251-8588 (JP)
(74) Representative: Cabinet Beau de Loménie
(86) International application number: PCT/JP2015/054383
(87) International publication number: WO 2015/125805

(56) References cited:
- EP-A1- 0 648 832
- EP-A1- 0 717 099
- EP-A1- 0 823 451
- EP-A1- 1 352 947
- EP-A1- 1 754 772
- EP-A2- 0 993 041
- JP-A- H0 959 664
- JP-A- H03 106 996
- JP-A- H07 102 274
- JP-A- H08 143 883
- JP-A- 2003 176 489
- JP-A- 2004 176 075
- JP-A- 2012 224 834
- US-B1- 6 352 961

## Description

### [Technical Field]

The present invention relates to a silicone composition and a lubricating use of this composition. More particularly, the invention relates to a silicone grease composition suitably used for the parts to be lubricated, to be more specific, the lubrication parts of the clutch, the torque limiter mechanism and the like where high coefficient of friction and excellent wear preventive characteristics are needed.

### [Background Art]

In consideration of the global environmental problems, weight reduction of the automobile has been advancing. In line with this tendency, a variety of portions tend to use more clutches and torque limiter mechanisms than ever. Of such a variety of clutches and torque limiter mechanisms using the grease composition in the automobile, the engine starter clutch is exposed to the highest torque and the severest operating conditions.

The clutch of the engine starter is composed of a clutch outer, a clutch inner, a roller disposed in a wedge-like space formed between the clutch outer and the clutch inner to transmit the rotation of the clutch outer to the clutch inner, and a spring which works to urge the roller toward the narrower side of the wedge-like space. When the clutch outer is rotated, the roller moves toward the narrower side of the wedge-like space and is then caught between the clutch outer and the clutch inner, thereby transmitting the rotation to the clutch inner (torque-transmitted state). Accordingly, the grease composition used for such portions requires a high coefficient of friction to prevent the slippage of the clutch outer, the clutch inner and the roller.

The following silicone grease compositions are conventionally known: a grease for the overrunning clutch (JP (Hei) 7-35824 B) where a base oil comprising a silicone oil has a coefficient of friction of 0.18 or more; grease compositions (JP (Hei) 5-230486 A and JP (Hei) 6-279777 A) comprising as the base oil organopolysiloxanes having a predetermined ratio of phenyl group or methyl group; and a traction grease composition (JP 2003-176489 A) comprising finely-divided particles of metallic oxide, a thickener, and a base oil containing a dimethyl silicone oil with a predetermined kinematic viscosity in an amount of 1 to 40 mass%. Those grease compositions make use of the advantages of the silicone oils that the coefficients of friction are high, and in addition, the surface tensions of the silicone oils range from 20 to 25 dyn/cm2, which are lower than those of other oils, so that a lubrication film may not readily be formed, thereby easily attaining to boundary lubrication.

A grease composition for a rolling bearing of JP H09-59664 A contains a silicone oil as a base oil and a magnesium compound and 0.5-120 wt% anticorrosive agent.

To prevent occurrence of brake noise when it is applied to a disk brake, JP 2012-224834 A teaches a grease composition containing a base oil and a thickener.

When the rotational speed of the clutch inner becomes higher than that of the clutch outer, the roller automatically moves toward a wider side of the wedge-like space as compressing the spring, thereby stopping the transmission of the rotation (torque non-transmitted state). Under such conditions, the clutch outer, the clutch inner and the roller reach a state of slippage due to generation of the relative rotation. In light of this, the grease composition used for such portions is required to have wear preventive characteristics.

### [Summary of Invention]

### [Technical Problem]

As previously explained, the clutch and the torque limiter mechanism are required to be smaller in size and lighter in weight in line with the recent tendency toward weight reduction in the automobile, and on the other hand, they are exposed to severer operating conditions. Especially, satisfactory torque transmission properties are demanded even when the operating conditions become more and more tough. For that reason, the grease composition is required to have a higher coefficient of friction. At the same time, the wear preventive characteristics are also needed when the grease composition is used for the clutch and the torque limiter mechanism.

Accordingly, an object of the invention is to provide a silicone grease composition having improved frictional characteristics, without deterioration of the wear preventive characteristics.

### [Solution to Problem]

A grease composition having an increased coefficient of friction without decrease of the wear preventive characteristics is obtained by adding as the friction modifier a metallic oxide with a Mohs hardness of 6 or less.

The invention is defined in the claims.

### [Effects of Invention]

According to the invention, a silicone grease composition where the frictional characteristics are improved without decrease of the wear preventive characteristics can be provided.

### [Description of Embodiments]

### <Base oil>

A silicone oil is used for the base oil in the grease composition according to the invention.

Specific examples of the silicone oil include dimethyl silicone oil, methylphenyl silicone oil (phenyl-modified silicone oil), methyl hydrogen silicone oil, polyether-modified silicone oil, aralkyl-modified silicone oil, fluoroalkyl-modified silicone oil, alkyl-modified silicone oil, fatty acid ester-modified silicone oil, and the like. Of the above silicone oils, dimethyl silicone oil and methylphenyl silicone oil are preferably used. The silicone oil represented by the following general formula (1) is particularly preferable:

(CH₃)₃SiO-[-Si(R1)(R2)-O-]n-Si(CH₃)₃ (1)

wherein R1 and R2 are each independently methyl group or phenyl group, the ratio of methyl group to the whole organic groups being 50 to 100 mol.%.

The kinematic viscosity of the silicone oil is not particularly limited, but may preferably be in the range of 20 to 10,000 mm²/s, more preferably 50 to 2,000 mm²/s at 25°C. When the kinematic viscosity of the silicone oil is less than 20 mm²/s, the base oil may easily separate from the grease. When the kinematic viscosity exceeds 10,000 mm²/s, the torque will increase at low temperatures due to the viscosity resistance. In any case, the results are practically undesirable.

In the above-mentioned formula (1), R1 and R2 are each independently methyl group or phenyl group, the ratio of the methyl group to the whole organic groups being 50 to 100 mol.%. When the molar ratio of the methyl group to the whole organic groups is less than 50 mol.%, the viscosity greatly varies depending on the temperature, and the pour point increases and the torque becomes large at low temperatures. The ratio of the methyl group to the whole organic groups may preferably be 60 to 100 mol.%, more preferably 80 to 98 mol.%, and still more preferably 90 to 95 mol.%.

The silicone oil may preferably be contained in an amount of 55 to 90 mass%, and more preferably 70 to 90 mass%, with respect to the total mass of the composition. Such a content of the silicone oil can favorably lead to high coefficient of friction.

The silicone oil may be used in combination with other base oil components so long as the performance of the silicone oil may not be impaired. One or more base oil components selected from the group consisting of mineral oils, poly α-olefins, polybutene, alkylbenzene, animal and vegetable oils, organic acid esters, diesters, polyol esters, polyalkylene glycols, polyvinyl ethers, polyphenyl ethers, and alkylphenyl ethers can be used. The amount of other base oil component(s) that can be used in combination with the silicone oil may preferably be 0 to 50 mass% with respect to the mass of the silicone oil used for the base oil. In order not to decrease the high coefficient of friction, the amount of other base oil component(s) may preferably be 0 to 20 mass%, more preferably 0 to 10 mass%, with respect to the mass of the lubricating base oil used in the invention. It is most preferable to use no other base oil component.

### <Thickener>

Soap type thickeners are lithium soaps and lithium complex soaps, urea type thickeners are diurea compounds, inorganic thickeners are organoclay and silica, organic thickeners are polytetrafluoroethylene and melamine cyanurate, and the like. The diurea compounds represented by the following general formula (2) may be used:

R3 -NHCONH-R4-NHCONH-R5 (2)

wherein R3 and R5 may be the same or different from each other, and R4 is a bivalent aromatic hydrocarbon group having 6 to 15 carbon atoms, so that the above-mentioned diurea thickener can be obtained by reacting a predetermined diisocyanate with a predetermined monoamine in the base oil. Specific examples of the preferable diisocyanate include diphenylmethane-4,4'-diisocyanate and tolylene diisocyanate. The monoamine includes aliphatic alicyclic amines, or the mixtures thereof, namely cyclohexylamine and octylamine, dodecylamine, hexadecylamine, octadecylamine, or a mixture thereof for preparation of the diurea thickener. The alicyclic aliphatic diurea compounds can be obtained by using cyclohexylamine together with dodecylamine, hexadecylamine, octadecylamine or the mixture thereof. Further, alicyclic aliphatic diurea compounds obtained from cyclohexylamine and octadecylamine, or the mixtures thereof are particularly preferable. A mixture of the following three kinds of diurea compounds represented by formula (2-1), (2-2) and (2-3) (where R is octadecyl group) is most preferable.

The content of the thickener, which may appropriately be adjusted in accordance with the desired consistency is generally 2 to 35 mass%, preferably 5 to 30 mass%, and more preferably 10 to 25 mass%.

When the content of the thickener is less than 2 mass%, the resultant product becomes a liquid, which cannot be used as a grease. When the content of the thickener exceeds 35 mass%, the resultant grease is not practically desirable because the grease is so hard that the torque will increase at low temperatures.

### <Friction modifier>

The grease composition of the invention comprises as the friction modifier a metallic oxide with a Mohs hardness of 6 or less.

The addition of the metallic oxide as the friction modifier can increase the coefficient of friction because the oil film becomes easy to break due to the metallic oxide entering into the surfaces to be lubricated. Even when the lubrication member is made of steel, use of the metallic oxide with a Mohs hardness of 6 or less can increase the coefficient of friction, with damage to the steel being minimized.

More specifically, magnesium oxide, potassium oxide, calcium oxide, scandium oxide, titanium oxide, vanadium oxide, chromium oxide, manganese oxide, iron oxide, cobalt oxide, nickel oxide, copper oxide, zinc oxide, gallium oxide, germanium oxide, strontium oxide, yttrium oxide, zirconium oxide, niobium oxide, molybdenum oxide, technetium oxide, ruthenium oxide, rhodium oxide, palladium oxide, silver oxide, indium oxide, tin oxide, antimony oxide, tellurium oxide, barium oxide, hafnium oxide, tantalum oxide, tungsten oxide, rhenium oxide, lead oxide, and silicon oxide can be used. Particularly, magnesium oxide, zinc oxide and molybdenum oxide are preferable. The Mohs hardness of the metallic oxide is preferably 6 or less, more preferably 2 to 6, and still more preferably 4 to 6. The Mohs hardness of more than 6 is not favorable because the abrasion will become harsh during the idling operation in the torque non-transmitted state.

The metallic oxide may preferably have an average particle diameter of 10 µm or less, more preferably 5 µm or less, and still more preferably 2 µm or less. When the average particle diameter exceeds 10 µm, it becomes difficult for the metallic oxide particles to come between the surfaces to be lubricated, and therefore a sufficient effect cannot be expected. The BET conversion method by N₂-adsorption may be used to determine the average particle diameter herein used.

The metallic oxide is contained in an amount of 0.1 to 10.0 mass%, preferably 0.3 to 7.0 mass%, more preferably 0.5 to 5.0 mass%, and most preferably 1.0 to 3.0 mass%, based on the total mass of the composition. When the content of the metallic oxide is less than 0.1 mass%, a sufficient effect cannot be expected. When the content of the metallic oxide exceeds 10.0 mass%, the cost will be disadvantageous because the effect is saturated.

### <Other additives>

Other additives conventionally used for grease, such as an antioxidant, rust inhibitor, metal deactivator, detergent dispersant, extreme pressure agent, antifoaming agent, demulsifier, oilness improver, solid lubricant and the like may be incorporated. Those auxiliary additives may be used alone or in combination. The auxiliary additives may be added if necessary, and in this case, the contents may be 0.01 to 10 mass% generally. However, the contents of those additives are not particularly limited as far as the effects of the invention are not degraded.

### <Consistency>

The grease composition of the invention may preferably have a worked penetration of 200 to 400, more preferably 230 to 380, and most preferably 250 to 350.

According to one preferable embodiment of the invention, the silicone grease composition comprises; a mixture of three kinds of diurea compounds represented by the above-mentioned formulas (2-1), (2-2) and (2-3) as a thickener, a base oil consisting of the silicone oil represented by the above-mentioned formula (1), with no other base oil component being added, and magnesium oxide, zinc oxide or molybdenum oxide as a friction modifier.

In the above embodiment, it is more preferable that the silicone grease composition comprise a mixture of three kinds of diurea compounds represented by the above-mentioned formulas (2-1), (2-2) and (2-3) as the thickener; the base oil consisting of the silicone oil represented by the above-mentioned formula (1) where R1 and R2 are each independently methyl group or phenyl group, with the ratio of methyl group to the whole organic groups being 50 to 100 mol.%, with no other base oil component being added; and magnesium oxide or zinc oxide or molybdenum oxide as the friction modifier, with the amount of the friction modifier being 0.1 to 10 mass% based on the total mass of the composition.

In the above embodiment, it is most preferable that the silicone grease composition comprise a mixture of three kinds of diurea compounds represented by the above-mentioned formulas (2-1), (2-2) and (2-3) as the thickener; the base oil consisting of the silicone oil represented by the above-mentioned formula (1) where R1 and R2 are each independently methyl group or phenyl group, with the ratio of methyl group to the whole organic groups being 95 mol.%, with no other base oil component being added; and magnesium oxide as the friction modifier, with the amount of the friction modifier being 1.0 to 3.0 mass% based on the total mass of the composition.

The silicone grease composition of the invention can be suitably used for the portions to be lubricated where a high coefficient of friction and excellent wear preventive characteristics are needed, to be more specific, the portions of clutch and torque limiter mechanism. More specifically, the silicone grease composition of the invention is usable for the overrunning clutch of automobile starters, the one way clutch of office equipment, a variety of traction driving mechanisms, and the like. Desirably, the surface of the portions to be lubricated may be a member made of steel.

### [Examples]

### <Preparation of silicon grease compositions>

### - Base oil

A silicone oil of formula (1) where R1 and R2 are each independently methyl group or phenyl group, with the ratio of methyl group to the whole organic groups being 95 mol.% was used.

### - Thickener

An alicyclic aliphatic diurea prepared from diphenylmethane-4,4'-diisocyanate, cyclohexylamine and octadecylamine was used.

### - Friction modifiers

Magnesium oxide (Mohs hardness: 5-6; Average particle diameter: 0.5 µm)
Zinc oxide (Mohs hardness: 4-5; Average particle diameter: 0.2 µm)
Molybdenum oxide (Mohs hardness: 2-3; Average particle diameter: 2.1 µm)
Titanium oxide (Mohs hardness: 7-8; Average particle diameter: 0.15 µm)
Boron nitride (Mohs hardness: 10; Average particle diameter: 4 µm)

Predetermined amounts of amines (i.e., cyclohexylamine and octadecylamine) were reacted with diphenylmethane diisocyanate in the base oil to prepare a base grease. By adding the base oil and other additives to the base grease, the resultant mixture was subjected to a milling treatment so as to have a worked penetration of 300 (JIS K2220), thereby obtaining a grease composition.

### <Test methods>

### - Low-speed and high-load friction test

In this test, the lubrication conditions of the clutch in the torque-transmitted state were assumed.

The test was conducted using a Falex test machine as prescribed in ASTM D2670. A test grease was applied to the journal and the blocks. A predetermined load was applied to both blocks against the journal in advance, and the test machine rotated the journal for one second. The generated frictional force was recorded, and then the initial coefficient of friction was determined 0.001 sec after starting. The test pieces and the test conditions are as shown below.
Journal: outer diameter 1/4n, SAE 3135 Steel, Rb 87-91
Blocks: AISI 1137 Steel, Rc 20-24
Contact pressure: 200 kgf/mm²
Circumferential speed: 0.096 m/sec

### - High-speed and Low-load abrasion test

In this test, the lubrication conditions of the clutch in the torque non-transmitted state were assumed.

The test was conducted using a LFW#1 test machine as prescribed in ASTM D2714. A load was applied to a roller against a ring. The test machine rotated the ring to determine the abrasion occurring on the roller using a micrometer. The test pieces and the test conditions are as shown below.
Ring: outer diameter 35 mm x width 8.7 mm, SAE 4620 Steel, Rc 58-63, RMS 6-12
Roller: Cylindrical roller for roller bearing, diameter 6 mm x 6 mm, SUJ-2
Contact pressure: 10 kgf/mm²
Circumferential speed: 12.8 m/sec

### <Evaluation criteria>

### - Low-speed and high-load friction test

### Coefficient of friction:

○○: 0.030 ≤ µ
○: 0.025 ≤ µ < 0.030
Δ: 0.020 ≤ µ < 0.025
×: µ < 0.020

### - High-speed and low-load abrasion test

### Depth of abrasion

○: < 6 mm
×: ≥ 6 mm

The results are shown in Tables 1 and 2. In the Tables, the amounts of the thickeners and the friction modifiers are expressed by mass%, which is based on the total mass of each grease composition. The balance is occupied by base oil.

**[Table 1]**

| | | Example 1 | | Example 2 | | Example 3 | | Example 4 | |
|---|---|---|---|---|---|---|---|---|---|
| Thickener Type | | Alicyclic aliphatic diurea | | Alicyclic aliphatic diurea | | Alicyclic aliphatic diurea | | Alicyclic aliphatic diurea | |
| Ratio | | 15 mass% | | 14 mass% | | 15 mass% | | 15 mass% | |
| Type of base oil | | Methylphenyl silicone | | Methylphenyl silicone | | Methylphenyl silicone | | Methylphenyl silicone | |
| Friction modifier | Type | Magnesium oxide, 1 mass% | | Magnesium oxide, 3 mass% | | Zinc oxide, 3 mass% | | Molybdenum oxide, 3 mass% | |
| | Mohs hardness | 5-6 | | 5-6 | | 4-5 | | 2-3 | |
| Coefficient of friction | | 0.031 | ○○ | 0.032 | ○○ | 0.028 | ○ | 0.022 | Δ |
| Depth of abrasion (mm) | | 4.0 | ○ | 4.1 | ○ | 5.5 | ○ | 3.5 | ○ |

**[Table 2]**

| | | Comparative Example 1 | | Comparative Example 2 | | Comparative Example 3 | |
|---|---|---|---|---|---|---|---|
| Thickener Type | | Alicyclic aliphatic diurea | | Alicyclic aliphatic diurea | | Alicyclic aliphatic diurea | |
| Ratio | | 15 mass% | | 15 mass% | | 16 mass% | |
| Base oil Type | | Methylphenyl silicone | | Methylphenyl silicone | | Methylphenyl silicone | |
| Friction modifier | Type | Titanium oxide 3 mass% | | Boron nitride 3 mass% | | - | |
| | Mohs hardness | 7-8 | | 10 | | - | |
| Coefficient of friction | | 0.020 | Δ | 0.030 | ○○ | 0.018 | x |
| Depth of abrasion (mm) | | 15.0 | x | 7.2 | x | 4.8 | ○ |

## Claims

1. A silicone grease composition comprising a thickener; a base oil comprising a silicone oil in an amount of 50 mass% or more of the total mass of the base oil; and a friction modifier comprising a metallic oxide with a Mohs hardness of 6 or less contained in an amount of 0.1 to 10 mass% based on the total mass of the composition, wherein the thickener is an alicyclic aliphatic diurea compound obtained from cyclohexylamine and dodecylamine, hexadecylamine, octadecylamine or a mixture thereof.

2. The silicone grease composition of claim 1, wherein the metallic oxide has a Mohs hardness of 2 to 6.

3. The silicone grease composition of claim 1 or 2, wherein the metallic oxide is magnesium oxide, zinc oxide or molybdenum oxide.

4. The silicone grease composition of any one of claims 1 to 3, wherein the silicone oil is represented by the following formula (1):
(CH₃)₃SiO-[-Si(R1)(R2)-O-]n-Si(CH₃)₃ (1)
wherein R1 and R2 are each independently methyl group or phenyl group, the ratio of methyl group to the whole organic groups being 50 to 100 mol.%.

5. The silicone grease composition of any one of claims 1 to 4, wherein the thickener is a mixture of the following three kinds of diurea compounds represented by formula (2-1), (2-2) and (2-3): wherein R is octadecyl group.

6. Use of a silicone grease composition according to any one of claims 1 to 5 for lubricating a portion between a clutch outer, a clutch inner and a roller of a clutch of an engine starter in an automobile.

## Patentansprüche

1. Silikonfettzusammensetzung, umfassend einen Verdicker; ein Grundöl, umfassend ein Silikonöl in einer Menge von 50 Masse-% oder mehr der Gesamtmasse des Grundöls; und einen Reibungsmodifizierer, umfassend ein metallisches Oxyd mit einer Mohs-Härte von 6 oder weniger, enthalten in einer Menge von 0,1 bis 10 Masse-%, auf der Grundlage der Gesamtmasse der Zusammensetzung, wobei der Verdicker eine alicyclische, aliphatische Di-Harnstoff-Verbindung ist, erhalten aus Cyclohexylamin und Dodecylamin, Hexadecylamin, Octadecylamin oder einem Gemisch daraus.

2. Silikonfettzusammensetzung gemäß Anspruch 1, wobei das metallische Oxyd eine Mohs-Härte von 2 bis 6 hat.

3. Silikonfettzusammensetzung gemäß Anspruch 1 oder 2, wobei das metallische Oxyd Magnesiumoxyd, Zinkoxyd oder Molybdänoxyd ist.

4. Silikonfettzusammensetzung gemäß irgendeinem der Ansprüche 1 bis 3, wobei das Silikonöl durch die folgende Formel (1) dargestellt wird:
(CH₃)₃SiO-[-Si(R1)(R2)-O-]n-Si(CH₃)₃ (1)
worin R1 und R2 jeweils unabhängig Methylgruppe oder Phenylgruppe sind, wobei das Verhältnis zwischen Methylgruppe und den ganzen organischen Gruppen von 50 bis 100 Mol-% ist.

5. Silikonfettzusammensetzung gemäß irgendeinem der Ansprüche 1 bis 4, wobei der Verdicker ein Gemisch aus den folgenden drei Sorten Di-HarnstoffVerbindungen ist, dargestellt durch die Formel (2-1), (2-2) und (2-3): worin Reine Octadecylgruppe ist.

6. Verwendung einer Silikonfettzusammensetzung aus irgendeinem der Ansprüche 1 bis 5 zum Schmieren eines Abschnitts zwischen einer Außenkupplung, einer Innenkupplung und einer Rolle einer Kupplung eines Anlassers in einem Automobil ist.

## Revendications

1. Composition de graisse de silicone comprenant un épaississant ; une huile de base comprenant une huile de silicone dans une quantité de 50 % en masse ou supérieure de la masse totale de l'huile de base ; et un agent de modification de friction comprenant un oxyde métallique avec une dureté Mohs de 6 ou inférieure contenu dans une quantité de 0,1 à 10 % en masse sur la base de la masse totale de la composition, dans laquelle l'épaississant est un composé de diurée aliphatique alicyclique obtenu à partir de cyclohexylamine et dodécylamine, hexadécylamine, octadécylamine ou d'un mélange de celles-ci.

2. Composition de graisse de silicone selon la revendication 1, dans laquelle l'oxyde métallique présente une dureté Mohs de 2 à 6.

3. Composition de graisse de silicone selon la revendication 1 ou 2, dans laquelle l'oxyde métallique est l'oxyde de magnésium, l'oxyde de zinc ou l'oxyde de molybdène.

4. Composition de graisse de silicone selon l'une quelconque des revendications 1 à 3, dans laquelle l'huile de silicone est représentée par la formule (1) suivante :
(CH₃)₃SiO-[-Si(R1)(R2)O-]n-Si(CH₃)₃ (1)
dans laquelle R1 et R2 sont chacun indépendamment le groupe méthyle ou le groupe phényle, le rapport de groupe méthyle à tous les groupes organiques étant de 50 à 100 % en mole.

5. Composition de graisse de silicone selon l'une quelconque des revendications 1 à 4, dans laquelle l'épaississant est un mélange des trois types suivants de composés de diurées représentés par les formules (2-1), (2-2) et (2-3) : dans lesquelles R est le groupe octadécyle.

6. Utilisation d'une composition de graisse de silicone selon l'une quelconque des revendications 1 à 5 pour la lubrification d'une portion entre un extérieur d'embrayage, un intérieur d'embrayage et un rouleau d'un embrayage d'un démarreur de moteur dans une automobile.
